

# UNITED STATES PATENT OFFICE.

ROBERT B. CARNAHAN, JR., OF MIDDLETOWN, OHIO, ASSIGNOR TO THE INTERNATIONAL METAL PRODUCTS COMPANY, OF NEWARK, NEW JERSEY.

## IRON MANUFACTURE.

940,784.

Specification of Letters Patent. Patented Nov. 23, 1909.

No Drawing.

Application filed July 16, 1909. Serial No. 507,911.

*To all whom it may concern:*

Be it known that I, ROBERT B. CARNAHAN, Jr., a citizen of the United States, residing at Middletown, Butler county, Ohio, have invented certain new and useful Improvements in Iron Manufacture, of which the following is a specification.

For the usual puddling and knobbling processes for the production of iron having certain qualities, the present invention substitutes a process by treating molten iron whereby there is obtained an iron combining in high degree a number of desired qualities not heretofore found in any single iron product.

The metal resulting from the improved method of production possesses an extraordinary high degree of malleability, it rolls into sheets remarkably free from blisters, it 20 galvanizes in a very superior manner, it resists corrosion to a superior extent, it yields a particularly smooth surface under the action of rolls, and it works readily at such low heats as to avoid the scaling of surfaces, 25 these combined qualities greatly reducing the percentage of waste.

The product of the process may take the form of rolling mill or bloomery ingots or foundry castings or further products worked 30 therefrom.

In carrying out my improved manufacture I charge a high-powered basic open-hearth furnace with pig-iron or cast iron or molten iron. In practice there has been substituted low carbon iron or steel scrap to a considerable extent, in some cases as high as eighty per cent of the charge. Lime or limestone is to be charged to reduce sulfur and phosphorus, these agents being preferably 35 charged prior to charging the metal. The charge is then to be refined as in making soft steel, by the employment of ore or agitation, or both, but, unlike the steel process, re-carburization at this stage is not necessary 40 in case the charge melts specially low in carbon. The refining operation is then to be carried forward with ascending temperature as the carbon becomes reduced, the refining being prolonged and at such high heat 45 (from one to four hours more time than is

employed in making high grade soft steel, and at an ultimate bath temperature of at least 2850 deg. F.) that, by bath test, the bath will contain not over .14 per cent. of sulfur, phosphorus, carbon, manganese and 55 silicon taken in the aggregate. For the best results it is desirable and practicable to reduce this aggregate to less than one half the percentage named, and to have neither carbon nor manganese over .02 per cent.

The refined metal is to be poured into molds while still at high temperature, and while still molten it is to be deoxidized and degasified to such extent that the resulting product will contain not over .05 per cent. of 60 oxygen as determined by the method of Lebedur, and preferably considerably below this, and will contain at least 99.80 per cent. of iron. The deoxidation and degasification may be very satisfactorily accomplished by 65 the addition of aluminum in the molten metal, say two and one-half pounds per ton. If done in the furnace it is recommended that aluminum pig-iron be used. Aluminum may be economized by partially deoxidizing the bath by employing pig-iron say 70 two to eight per cent. of the charge. The degasifying and deoxidizing agents must, of course, not be such as to lessen the above mentioned purity of the ultimate product. 75 In tapping the metal the slag is floated off and the product is thus freed from it.

Among the various methods for oxygen determination that of Lebedur has been chosen on account of its superior reliability 80 and accuracy, and is herein mentioned as a standard in view of the differing results arrived at by various methods.

I claim:

The improved manufacture of rolling mill 90 and bloomery ingots and foundry castings consisting of the following steps:—charging a high-powered basic open-hearth furnace with iron; employing therewith eliminating agents for carbon and manganese and 95 sulfur and phosphorus; refining the charge in molten condition at such high and increasing heat and for such prolonged period that analysis by bath test shows that the sulfur, phosphorus, carbon, manganese and silicon 100

con are not over .14 per cent. when taken in the aggregate; and pouring the hot purified metal into molds, and treating the metal while in molten state with a deoxidizing and 5 degasifying agent or agents to such extent that the product will contain not over .05 per cent. of oxygen and will contain at least

99.80 per cent. of iron, substantially as set forth.

ROBERT B. CARNAHAN, JR.

Witnesses:

ELMER R. SHIPLEY,  
M. S. BELDEN.